

April 30, 1946.

M. H. FURLAUD

2,399,178

## PROCESS FOR THE TREATMENT OF BERYL

Filed Feb. 9, 1945



*INVENTOR.*

Maxime H. Furlaud

BY  
  
Robert W. Dinsmore  
ATTORNEY

## UNITED STATES PATENT OFFICE

2,399,178

## PROCESS FOR THE TREATMENT OF BERYL

Maxime H. Furlaud, Buenos Aires, Argentina

Application February 9, 1945, Serial No. 577,121

19 Claims. (Cl. 23—16)

This invention relates to a process for the production of beryllium compounds from minerals, especially beryl. More particularly, the invention relates to the recovery of the beryllium values in such minerals by the selective fluorination of the beryllium therein so that the separation of the beryllium values from the other constituents in the minerals is very materially simplified.

While there have been many investigators who have proposed various processes for decomposing or "opening up" beryl with several different fluorine compounds, these processes have been burdened with one or more of the following disadvantages: multiple process steps, expensive reagents, heavy consumption of reagents, impurities in the recovered beryllium values, and the like. Furthermore, from the commercial viewpoint none of these processes have been amenable to continuous operation and, therefore, they have also been handicapped by the wastes and expenses inherent in batchwise operations.

A primary object of this invention is to provide a simple and direct method of recovering the beryllium values in minerals.

Another principal object is to "open up" beryllium-containing minerals by a process involving a minimum consumption of chemical reagents.

A further object of my invention is to obtain from beryllium minerals beryllium compounds in a high state of purity.

Still another object is to provide a commercially feasible process for treating beryllium minerals, either batchwise or continuously, as may appear best in each installation in the light of surrounding circumstances.

Other objects of my invention will become apparent from the description which follows.

In accordance with my invention, beryllium-containing minerals, e. g., beryl and phenacite, in finely divided form are treated with ammonium fluorides, viz: neutral ammonium fluoride ( $\text{NH}_4\text{F}$ ) and ammonium acid fluoride ( $\text{NH}_4\text{F}\cdot\text{HF}$ ), in vapor form under reaction conditions while maintaining the powdered mineral in a fluidized state.

The use of the fluidization technique in my process is of fundamental importance in achieving a new and surprising effect, i. e., selective fluorination of beryllium in spite of the presence in the mineral of the other constituents, aluminum and silicon, which are reactive to fluorinating reagents. I have found that the intimate contact which obtains in fluidizing finely divided beryllium minerals with a vaporized ammonium fluoride leads to rapid fluorination of the beryllium constituent throughout the entire mass of

powdered mineral. Under these circumstances, it is possible to fluorinate the beryllium present in the mineral substantially completely without significant attack of the other mineral constituents.

5 This is all the more surprising since it is known that the rate of fluorination of beryllium oxide is only slightly greater than that of either alumina or silica. The most common beryllium mineral is beryl which is represented by the formula,

10  $3\text{BeO}\cdot\text{Al}_2\text{O}_3\cdot 6\text{SiO}_2$   
It has not heretofore been possible to take advantage of this slight difference in reactivities in order to obtain an efficient separation of beryllium 15 from the other constituents of the mineral. The secret of the success of the present invention appears to rest in presenting to every fluorine atom an opportunity of reacting with the preferred beryllium atom, an opportunity which was not 20 given in prior processes.

On the basis of this discovery, I control the selective fluorination of beryllium in my process by limiting the quantity of ammonium fluoride used up to that quantity which according to 25 theory is just enough to react with all of the beryllium present in the mineral undergoing treatment. In other words, the fluorinating reagent is consumed in stoichiometrical proportions with respect to beryllium. In batchwise operation, this 30 is accomplished by passing vaporized ammonium fluoride through the fluidized batch of mineral until that quantity of reagent has reacted, which by prior analysis of the mineral for beryllium content and by calculation is just enough to convert 35 all of the beryllium present to beryllium fluoride ( $\text{BeF}_2$ ).

In continuous operation the powdered mineral is fed to the reactor at a rate stoichiometrically equivalent (with respect to beryllium) to the rate 40 of consumption of ammonium fluoride in the reactor. Powdered reaction product containing equivalent beryllium fluoride is continuously withdrawn.

Conditions must further be set so that the 45 beryllium oxide in the mineral is substantially completely converted to beryllium fluoride and so that the ammonium fluoride is consumed economically. In adjusting these conditions it is well to remember that both the horizontal cross-section 50 of the reactor and the linear velocity of the vapors ascending through the reactor are fixed by other considerations; the latter by inherent requirements of the fluidizing technique which will be described hereinbelow and the former by the 55 desired productive capacity of the reactor as re-

lated to the vapor velocity. It develops, then, that the economical consumptions of the mineral and the ammonium fluoride are related to the depth of fluidized bed which is established in the reactor and that the depth must be chosen to accommodate whichever of these demands requires the greater depth, that is, the greater exposure time to the opposite reactant.

The exposure time required by the reagent vapor is determined by performing experiments in which the selected ammonium fluoride is passed up through a bed of comminuted mineral in which the beryllium content has been nearly completely converted to beryllium fluoride, say about 95% of the beryllium content has been fluorinated. The depth of fluidized bed needed is then calculated from the experimentally determined exposure time for the ammonium fluoride and from the gas linear velocity chosen within the limits set forth hereinbelow.

The exposure time required by the mineral is determined experimentally by reacting a thin layer of powdered mineral with vapor containing various proportions of the selected ammonium fluoride and gaseous reaction products (ammonia and water vapor) and by observing the rate of conversion of the mineral in each case. From these data the time to convert a particle of mineral under the average conditions prevailing in a fluidizing reactor may be calculated. The actual exposure time of the mineral must be made considerably longer, say ten times longer, than the calculated average time to react to avoid short-circuiting of unreacted particles from the inlet to the outlet of the reactor.

The calculated exposure time of the mineral is realized by regulating the ratio of the holdup of mineral in the reactor to the throughput of mineral per unit of time. For example, if a reactor holds 200 lbs. of mineral and the throughput is 200 lbs. per hour, the exposure time is 1 hour. The required holdup as related to the cross-section of the reactor, which has been fixed by deciding upon a desired productive capacity and vapor velocity, gives a second required depth of bed. This bed depth or that calculated from consideration of the consumption of the vaporized reagent, whichever is the greater of the two, is incorporated in the practical design of the fluidizing reactor.

Where the solid reacts with unusual rapidity, it may be found that the inlet and outlet of the reactor may be located far enough apart to prevent the flow of particles from the one opening to the other before they have reacted. This is desirable but a fortuitous and unusual occurrence.

In general, the linear velocity of the vapors is made to fall in the range of about 0.1 to 5.0 feet per second, preferably about 0.5 to 2.0 feet per second. With suitable precautions, somewhat higher or lower velocities may be employed. Such vapor velocities ensure good fluidization of beryllium minerals which have been pulverized to particle sizes in the approximate range of 100 to 400 mesh; preferably at least about 60% of the comminuted mineral should pass through a 200-mesh screen. Good fluidization, in turn, is highly conducive to the selective fluorination of the beryllium mineral as well as to the usual attributes of the technique, e. g., uniform temperature throughout the reaction mass.

While for the sake of clarity and ease of presentation the foregoing description has stressed that in accordance with my invention,

a powdered mineral, e. g., beryl, is treated with a vaporized ammonium fluoride under such conditions that the beryllium content is substantially completely converted to beryllium fluoride,

- 5 it is obvious to those skilled in the art that it is practical and indeed advisable to limit the fluorination to a maximum of about 95% of the beryllium content of the mineral. Particularly in large-scale operations, such a precaution 10 leads to the recovery of high-purity beryllium fluoride; the small loss of the beryllium content is a small price for avoiding the presence of impurities, such as aluminum fluoride, which tend to be formed when an effort is made to drive 15 the selective fluorination of beryllium to completeness with respect to beryllium. It should also be noted that while it has been stated that the fluorinating reagent is consumed in substantially stoichiometrical proportions with respect to the beryllium content, this is not to say 20 that an excess of the reagent may not be passed through the reaction mass. In view of the fairly low cost of the reagents contemplated in my invention, reasonable excesses of such reagents 25 which pass through the fluidized mass without reaction can easily be permitted, especially in systems in which the fluorinating reagents are recovered and reused as shown hereinafter.

Suitable fluorination temperatures are well 30 known in the technical literature but I generally operate my process at temperatures in the range of about 350° to 700° C., preferably about 450° to 600° C. Similarly, atmospheric pressure is commonly employed but in some cases an 35 elevated pressure may be favored.

A further aspect of my invention is the rapid conversion of beryllium fluoride to beryllium oxide, when the latter compound is preferred as the starting material in processes for the production of beryllium metal. My novel procedure for converting beryllium fluoride to beryllium oxide involves introducing the fluoride, as either a solution or a solid, in a discrete form into a fluidized hot mass of particulate beryllium oxide. 40 The mass of oxide is maintained in a fluidized state by the passage therethrough of steam supplied to the reactor as such or in the form of an aqueous solution of the beryllium fluoride which is charged to the reactor. A generous excess of 45 steam is advisable since it favors the conversion of beryllium fluoride to beryllium oxide. While atmospheric pressure is ordinarily used, a reduced pressure favors the conversion of the fluoride to the oxide. Suitable temperatures for 50 this conversion lie in the range of about 300° to 700° C., preferably about 400° to 600° C. Gas velocities and particle sizes for this fluidizing reactor are similar to those hereinabove discussed for the fluorination reactor.

60 For more detailed description and further clarification of my invention, reference is had to the accompanying drawing which schematically illustrates a preferred form of the process embodying continuous operation and several other 65 features of my invention.

In the drawing, an upright cylindrical reactor 1 has a tapered bottom 2 to which is attached pipe 3 for introducing the fluorinating reagent, e. g., ammonium acid fluoride. As shown, the 70 ammonium acid fluoride passes through a vaporizer 4. Thence, the fluoride vapors flow through pipe 3 into reactor 1 wherein they fluidize a mass of powdered mineral, say beryl, and at the same time react with the beryl particles, 75 converting the beryllium oxide of the mineral into

beryllium fluoride. In the course of this reaction, the ammonium acid fluoride vapors are changed to ammonia and water vapor. These transformations are represented by the equation:



The fluidized reaction mass within reactor 1 is maintained at the desired reaction temperature, say 600° C., by burning a combustible mixture such as natural gas and air in a plurality of fire-tubes 5 disposed within the reactor 1. The flue gases from these fire-tubes are vented to the atmosphere. Fluidization of the powdered mass is conductive to a rapid transfer of heat from fire-tubes 5 to the reaction mass as well as to a uniform reaction temperature. The reaction gases, very largely ammonia and water vapor, and perhaps small quantities of the fluorinating reagent vapors which have not reacted, become separated from the fluidized mineral mass at the pseudo-liquid level 6 and emerge from reactor 1 through pipe 7. Generally, there is a tendency for a small proportion of the powdered mineral to become entrained in the gases leaving reactor 1; a filter, cyclone separator or similar device may be interposed in pipe 7 to separate the particles from the gases so that they may be returned to reactor 1. Alternatively, the entrained solids are recovered from the gases after the latter have been liquefied in condenser 8. Discharging into condenser 8 from pipe 9 is a stream of hydrogen fluoride and water vapor. The mixed streams from pipes 8 and 9 form an aqueous solution of ammonium acid fluoride through condensation. The fluoride solution flows through pipe 10 to evaporator 11 wherein water is expelled from the solution. The ammonium fluoride is then moved along line 12 to vaporizer 4 whence the fluorinating reagent vapors return to reactor 1 to attack fresh mineral particles.

At a rate commensurate with the introduction of fluorinating reagent vapors, there is admitted into reactor 1 fresh, powdered beryl. The pulverized beryl is charged into feed hopper 14 and from there the powder flows down standpipe 15 and through controlling slide valve 16 into reactor 1. The powder in this feed system is maintained in a free-flowing condition by passing a small quantity of fluidizing gas, such as air or steam, up through the powdered mass. A tube 17 for introducing such a gas is shown above slide valve 16.

Keeping pace with the addition of fresh mineral is the withdrawal of reacted mineral. The reacted mineral particles flow out of reactor 1 by way of standpipe 18 and slide valve 19 or equivalent flow-regulating device, e. g., a star-feeder. A tube 20 above valve 19 serves to introduce air or other convenient gas to prevent the packing of mineral powder within pipe 18.

The reacted solids are discharged into a solution tank 21 wherein with the aid of water the beryllium fluoride formed in reactor 1 is dissolved from the other mineral constituents, chiefly alumina and silica, which are not soluble in water. The resultant slurry proceeds through pipe 22 to a suitable filter 23, such as an Oliver rotary filter, which separates the insoluble material, viz: alumina, silica, etc., from the beryllium fluoride solution. The fluoride solution is transported by way of pipe 24 and pump 25 to fluidizing reactor 26. Preferably, the solution is introduced through an atomizing nozzle 27. If desired, the beryllium fluoride solution may be concentrated by evaporation of water and preheated before entering

reactor 26. To maintain a desired reaction temperature, say 550° C., reactor 26 is enclosed by a furnace setting 28 in which a fuel like gas or oil is fired. Reactor 26 contains a fluidized mass of powdered beryllium oxide which is formed therein by the reaction between beryllium fluoride and steam. The steam may be introduced from an external source or it may be generated from the aqueous solution of beryllium fluoride entering reactor 1 by way of nozzle 27. Steam disappearing in reactor 26 because of reaction with beryllium fluoride is replaced by hydrogen fluoride (HF) resulting from the same reaction. The reaction is represented by the equation:



Comminuted beryllium oxide which forms the fluidized bed with pseudo-liquid level 29 flows into standpipe 30 from which it is discharged at a rate equal to the rate of its formation within reactor 26. The rate of withdrawal is controlled by slide valve 31 or its equivalent. A fluidizing tube 32 above valve 31 serves to introduce steam to prevent packing of the oxide powder within standpipe 30. The reaction gases of reactor 26, very largely hydrogen fluoride and excess steam, become separated from the fluidized bed of beryllium oxide at pseudo-liquid level 29. Entrained oxide particles may be removed from the effluent gases by inserting a suitable separator, like a cyclone or a Cottrell precipitator, in pipe 9 or they may be recovered from the condensate after the gases have passed through condenser 8. As hereinabove mentioned, the gases flowing through pipes 7 and 9 intermingle within condenser 8; reaction occurs and an aqueous solution of ammonium acid fluoride emerges as condensate. The equation of the reaction between the gas streams of pipes 7 and 9 is:



As a specific example of the foregoing embodiment of my process, an installation designed to treat 200 lbs. of beryl per hour will be considered. In this case, reactor 1 has an inside diameter of 11 inches and pseudo-liquid level 6 is 20 feet above the bottom of reactor 1. A temperature of 600° C. is maintained in the fluidized mass of reactor 1 by three fire-tubes 5. The fire-tubes are 2 inches in diameter and consume about 0.3 gallon of oil per hour per tube. For fluorination, ammonium acid fluoride passes through vaporizer 4 and the resultant vapors at a temperature of 500° C. are admitted into reactor 1 at a rate such that the gas linear velocity up through reactor 1 is about 1 foot per second. Powdered beryl, about 80% passing through a 200-mesh screen, is fed to reactor 1 at the rate of 200 lbs. per hour, while the treated mineral is withdrawn at a commensurate rate (about 218.5 lbs. per hour). The steps of dissolving, filtering, etc. the treated mineral are simple, conventional operations for which no numerical data are given here for the sake of brevity. Reactor 26 for converting beryllium fluoride to oxide is 14 inches in internal diameter. The furnace setting 28 maintains the fluidized mass in reactor 26 at a temperature of 580° C. A 50% solution of beryllium fluoride is atomized into reactor 26 through nozzle 27 at a rate to establish a gas linear velocity of about 1 foot per second up through the reactor. Under the conditions maintained in reactor 26, the fine droplets of beryllium fluoride solution are flashed to steam and residual particles of beryllium fluoride; in turn, the steam reacts with the beryllium fluoride to form beryllium oxide.

lum fluoride particles to yield particulate beryllium oxide and gaseous hydrogen fluoride. Beryllium oxide powder is withdrawn from reactor 26 in the vicinity of its pseudo-liquid level 29 which is approximately 20 feet above the bottom of reactor 26. The rate of withdrawal is about 21 lbs. of beryllium oxide per hour. Accordingly, it is obvious from the data of this example that with simple and inexpensive equipment my process is capable of continuously recovering from beryl beryllium oxide which is free of objectionable impurities; furthermore, the process involves a low expenditure of energy and no consumption of chemical reagent (other than accidental losses) since the ammonium fluoride used is regenerated and recycled constantly.

While the process of my invention has been described hereinabove in considerable detail in terms of the preferred embodiment which includes regeneration and recycling of the fluorinating reagent, conversion of an aqueous solution of beryllium fluoride to finely divided beryllium oxide, and continuous operation, it is understood that the process may be conducted batchwise, or beryllium fluoride may be fed to electrolytic cells to produce beryllium metal without going through the step of making beryllium oxide, or any of several similar modifications may be followed, as evaporating beryllium fluoride to its oxyfluoride.

Similarly, beryllium fluoride produced by any method, e. g., by complete fluorination of powdered beryl and by chemical separation of the mixed fluorides, may be converted to beryllium oxide by my fluidizing process. The particulate beryllium oxide formed in my process is well suited for charging into an arc furnace wherein the oxide, admixed with powdered carbon and powdered copper or copper oxide, is reduced to beryllium-copper alloy. Beryllium is commonly produced in the form of its copper alloy.

Briefly, then, my invention contemplates the selective fluorination of the beryllium constituent in a mineral by fluidization with ammonium fluoride vapors and the conversion of beryllium fluoride to beryllium oxide by fluidization with steam, said operations being carried out jointly or separately, and batchwise or continuously.

Those skilled in the art will appreciate that my invention is amenable to many variations without departing from its spirit or intent. For example, fluidizing reactors 1 and 26 have been depicted for so-called overflow or bottom withdrawal of powdered solids but overhead removal of solids by entrainment in the gases leaving a reactor is known and feasible. In the latter case, the solids would be recovered from the reaction gases by conventional separators like cyclones and electrical precipitators.

The fluidizing technique employed in the process of my invention has found extensive application in the petroleum refining industry and is described in many articles in the literature, for instance Chemical and Metallurgical Engineering, June 1944, pages 94 et seq.

It is known that under certain conditions of evaporation and concentration of aqueous solutions of beryllium fluoride the fluoride changes to the oxyfluoride. Where it is stated in the specification or appended claims that beryllium fluoride is recovered from the fluorinated mineral or is treated with steam to yield the oxide, those skilled in the art will appreciate that the beryllium fluoride may be partly or wholly in the form of beryllium oxyfluoride. Accordingly, in the

claims, the term, beryllium fluoride, should be interpreted broadly as meaning beryllium fluoride as such or as the oxyfluoride or as a mixture of the two.

5 It is well to note that while with my fluidization process the conversion of beryllium fluoride with steam to beryllium oxide can be driven to completeness, the withdrawal of incompletely reacted solids from the fluidizing reactor is permissible. In such case, the solids are washed with water to dissolve away residual beryllium fluoride and to leave behind substantially pure beryllium oxide as product. The wash water containing beryllium fluoride may be used to dissolve additional beryllium fluoride in solution tank 21 or it may be recycled directly to reactor 26.

What I claim is:

1. In the process of recovering beryllium from a beryllium-containing mineral, the step of selectively fluorinating said mineral in respect to beryllium by injecting an ammonium fluoride in vapor form into a fluidized mass of said mineral maintained at reaction conditions.

2. The process of claim 1 wherein the beryllium-containing mineral is beryl.

3. The process of claim 1 wherein the reaction conditions include a temperature in the range of about 350° to 700° C.

4. The process of selectively fluorinating a beryllium-containing mineral in respect to beryllium, which comprises exposing said mineral in finely divided form to vapors of an ammonium fluoride at reaction conditions and for a period of time not exceeding that which is just sufficient to convert the beryllium content of said mineral to beryllium fluoride, while maintaining said finely divided mineral in a fluidized state.

5. The process of claim 4 wherein the reaction conditions include a temperature in the range of about 350° to 700° C.

6. The process of claim 4 wherein the exposure period is sufficient to convert only about 95% of the beryllium content of the mineral.

7. The continuous process for recovering the beryllium content of beryl, which comprises simultaneously introducing powdered beryl and vaporized ammonium acid fluoride into a reactor in which a fluidized mass of beryl is established and maintained at reaction conditions, and withdrawing reaction gases and solids therefrom, the withdrawal of said reaction solids being controlled so that the amount of fluorination does not exceed that which is just sufficient to convert the beryllium content of said powdered beryl to beryllium fluoride.

8. The process of claim 7 wherein the reaction gases flowing up through the fluidized mass have a linear velocity in the range of about 0.5 to 2.0 feet per second.

9. The process of claim 7 wherein the reaction conditions include a temperature in the range of about 450° to 600° C.

10. The process of producing beryllium oxide from finely divided beryllium-containing mineral, which comprises selectively fluorinating said mineral in respect to beryllium by passing an ammonium fluoride in vapor form through a fluidized mass of said mineral maintained at reaction conditions, separating the resultant beryllium fluoride from the thus fluorinated mineral, and converting said beryllium fluoride to beryllium oxide by treating said beryllium fluoride in comminuted form with steam under reacting and fluidizing conditions.

11. The process of claim 10 wherein the steps

of selectively fluorinating the beryllium-containing mineral and of converting beryllium fluoride to beryllium oxide are conducted continuously and the effluent gases from said steps are combined to regenerate ammonium fluoride for recycling to the fluorinating step.

12. The continuous process of producing beryllium oxide from finely divided beryl, which comprises selectively fluorinating said beryl in respect to beryllium by passing vaporized ammonium acid fluoride at a linear velocity in the range of about 0.5 to 2.0 feet per second through a fluidized mass of said beryl maintained at a temperature in the range of about 350° to 700° C., separating the resultant beryllium fluoride from the thus fluorinated beryl, and converting said beryllium fluoride to beryllium oxide by treating said beryllium fluoride in comminuted form with steam in a fluidizing reactor through which the reaction gases flow at a linear velocity in the range of about 0.5 to 2.0 feet per second and in which the temperature is in the range of about 300° to 700° C.

13. The process of claim 12 wherein the finely divided beryl is of such particle size that at least 60% of the material passes through a 200-mesh screen and the selective fluorination is controlled so as to react not more than about 95% of the beryllium content of said beryl.

14. The process of converting beryllium fluoride into beryllium oxide, which comprises introducing said fluoride in discrete form into a fluid-

izing reactor, maintaining fluidization in said reactor while reacting steam with said fluoride, and withdrawing the gaseous and solid products of reaction.

15. The process of claim 14 wherein the reaction between steam and beryllium fluoride is conducted at a temperature in the range of about 300° to 700° C.

16. The process of claim 14 wherein fluidization is maintained by permitting the reaction gases to flow up through the reactor at a linear velocity in the range of about 0.5 to 2.0 feet per second.

17. The process of converting beryllium fluoride to beryllium oxide, which comprises establishing a fluidized bed of comminuted beryllium oxide, maintaining said bed at a temperature in the range of about 300° to 700° C., atomizing an aqueous solution of beryllium fluoride into said bed, and withdrawing reaction gases and comminuted beryllium oxide from said bed at a rate commensurate with the rate of formation of beryllium oxide through atomization of said solution into said bed.

18. The process of claim 17 wherein the comminuted beryllium oxide is of such particle size that at least 60% of the material passes through a 200-mesh screen.

19. The process of claim 17 wherein the aqueous solution of beryllium fluoride is of about 50% concentration.

MAXIME H. FURLAUD.